

April 28, 1964

W. C. RICHARDSON ETAL

3,131,076

PROCESS FOR MAKING CELLULOSE SPONGE

Filed May 4, 1961

2 Sheets-Sheet 1



INVENTORS

WILLIAM C. RICHARDSON  
RICHARD J. BOHNHOFF  
BY THEIR ATTORNEYS

*Howard and Howard.*

April 28, 1964

W. C. RICHARDSON ETAL

3,131,076

PROCESS FOR MAKING CELLULOSE SPONGE

Filed May 4, 1961

2 Sheets-Sheet 2



INVENTORS

WILLIAM C. RICHARDSON  
RICHARD J. BOHNHOFF  
BY THEIR ATTORNEYS

*Howson and Howson.*

1

3,131,076

**PROCESS FOR MAKING CELLULOSE SPONGE**  
William C. Richardson, Mobile, and Richard J. Bohnhoff,  
Loxley, Ala., assignors, by mesne assignments, to  
Courtaulds, Limited, London, England, a British  
company

Filed May 4, 1961, Ser. No. 107,838  
1 Claim. (Cl. 106—122)

This invention relates to the manufacture of cellulose sponge and in particular to a method for making cellulose sponge of improved strength.

Cellulose sponge is conventionally made by mixing together viscose, a crystalline pore forming material, and cellulose fiber. The pasty mixture is then placed in a mold and heated. The viscose is regenerated, and the crystalline pore former is melted or dissolved, leaving the sponge product.

The function of the fibers in the sponge mix is to provide strength and cohesiveness. To do this, however, the fibers must be evenly dispersed throughout the original viscose. Unfortunately it has been found that when the fibers are put into the viscose they do not disperse, but on the contrary tend to agglomerate and form clumps.

To overcome this tendency it has been proposed to add complex wetting and dispersing agents to the viscose. However, such agents are expensive and may have an undesirable effect on the finished product.

It is well known that cellulosic fibers swell in various reagents such as caustic soda, zinc chloride, and the like. It is also known that the degree of swelling is a function of the specific fiber treated, the swelling agent used and the swelling agent concentration. Further it has been found that for any particular fiber and swelling agent there is a concentration of swelling agent at which maximum swelling of the fiber occurs.

Now viscose, which is an alkaline medium containing free NaOH, is itself a swelling agent for cellulose. However, viscose normally used for sponge-making contains not more than say 10% total NaOH, i.e. free and combined as sodium cellulose xanthate of which not more than about 7% will be free. Usually the viscose will contain on the order of 4 to 8% total NaOH of which say 1% to 5% will be free NaOH. Such concentrations are not high enough to effect maximum swelling of cellulose fibers, and as noted above when fibers are put into normal viscose they tend to form clumps and aggregates. It has now been discovered, however, that when the swelling agent concentration is raised to a level corresponding to the concentration at which maximum swelling of the fibers in the viscose occurs, a smooth fiber dispersion is obtained and sponge products having improved strength result.

The invention therefore comprises, in a process for making cellulose sponge wherein viscose, cellulose reinforcing fibers and a pore-forming substance are combined to form a sponge mix, which is thereafter coagulated and regenerated to form a sponge structure, the improvement which comprises adding a swelling agent to the mix to give a concentration corresponding approximately to the concentration at which maximum swelling occurs. Normally the swelling agent concentration used

2

will be within 1% ( $\pm$  1%) of the concentration at which maximum swelling occurs.

In the drawings:

FIG. 1 is a graph showing the effect of swelling agent concentration in viscose on the swelling of cotton fiber and the tenacity of sponge made therefrom.

FIG. 2 is a graph showing the effect of swelling agent concentration in viscose on the swelling of ramie fiber and the tenacity of sponge made therefrom.

As noted above, conventional cellulose sponge paste contains viscose, reinforcing fiber and a pore forming agent.

The viscose may be any conventional type customarily used for fiber forming purposes. It will usually, but not necessarily, contain 5-9% by weight cellulose, and 4.5-6.5% by weight total NaOH. It may be aged or unaged, and have a gamma number of say 20 to 50.

The fiber used may be any cellulosic fiber, normally a natural cellulosic fiber such as cotton, ramie, jute or flax.

The pore forming agent is conventionally sodium sulfate. Glauber's salt ( $Na_2SO_4 \cdot 10H_2O$ ) is normally used, though the anhydrous salt may also be used if desired. There is, however, no advantage in using the anhydrous material. In place of sodium sulfate, other fusible, water soluble salts that do not readily regenerate viscose may be used, as may gas forming substances such as aluminum powder.

The cellulose swelling agent may be any of a large variety of materials including the alkali metal hydroxides, the alkali metal salts of weak acids, e.g. sodium zincate, salts of weak bases and strong acids such as zinc chloride and zinc nitrate and the like. Sodium hydroxide is, however, much preferred since it is a very effective swelling agent and introduces no new elements into the sponge making mixture.

The proportions of viscose, fiber and pore forming material in the mixture may vary within wide limits. In general, however, for one part by weight of viscose, between about 0.05 and about 0.15 part of fiber and about 2 to 7 parts of pore forming agent are used.

The particle size of the pore forming agent is not especially critical and will depend to some extent on the size of the pores desired. A normal range would be from say fine dust to  $\frac{1}{2}$ ".

As noted above, the concentration of swelling agent at which maximum swelling occurs, depends on the fiber and the agent. In the case of caustic soda, with most natural cellulose fibers, maximum swelling is obtained in viscose containing from 9 to 12% free NaOH.

In carrying out the invention it may be desirable to determine the maximum swelling concentration for the particular fiber, viscose and swelling agent to be used. This may be done by taking samples of the fiber, loading the individual fibers with an appropriate weight, immersing the fibers in viscose containing varying amounts of the swelling agent for say 30 minutes and then measuring the length of fiber. As Marsh (Mercerization, Chapman-Hall, London, 1941) has shown, longitudinal contraction is an index of cross-sectional swelling and the concentration of swelling agent which gives maximum contraction corresponds to the concentration for maximum swelling.

The procedural steps necessary to make sponge in accordance with the invention are entirely conventional.

The viscose and swelling agent are normally mixed together and the fiber then added. As the fiber is added to the viscose and swelling agent the effect of reaching a maximum swelling is clearly visible. Clumps of fiber break up and a smooth dispersion is obtained.

The form in which the swelling agent is added is not of major significance. Preferably, however, it is added as an aqueous solution of moderate concentration, say 25 to 50%, by weight. The viscose-fiber mass is normally highly viscous and the additional water aids in obtaining an even mixture without excessive stirring as well as avoiding high local concentrations of swelling agent. On the other hand, too much water is undesirable in causing dissolution and waste of pore former. Generally not more than about 0.15 parts of water, per part of viscose is added with the swelling agent.

After mixing, the paste or mix is put into a mold or poured on a slab and heated to say 90 to 100° C. to regenerate the viscose. After regeneration the sponge is washed thoroughly to remove pore former and is then ready for use.

The invention will be further described by means of the following specific examples which are given for purposes of illustration only and are not to be taken as in any way limiting the invention beyond the scope of the appended claim.

#### EXAMPLE I

To samples of viscose containing 8.75% cellulose and 5.0% NaOH (3.0% bound NaOH) were added varying amounts of NaOH as a 50% aqueous solution to give free caustic concentrations varying from about 5 to about 13% by weight. Cotton fibers approximately 2.5 cm. long were loaded with 50 mg. weights and immersed in the viscose samples for 30 minutes. The change in length was measured in situ. The contraction divided by the original length  $\times 100$  was recorded as percent contraction and appears in the appropriate column of Table 1 below.

Viscose samples containing varying amounts of NaOH were next used to make sponge. The mix was prepared by adding the required amount of sodium hydroxide as 50% aqueous solution to the viscose, while stirring. The fibers were next added in the proportion of 0.07 part by weight of fiber to one part of viscose. Finally the sodium sulphate ( $\text{Na}_2\text{SO}_4 \cdot 10\text{H}_2\text{O}$ ) was added, using a particle size through a 0.635 cm. sieve. About 5 parts of  $\text{Na}_2\text{SO}_4 \cdot 10\text{H}_2\text{O}$  were used per part of viscose. After the paste was thoroughly kneaded it was placed in stainless molds lined with polyethylene and having perforated bottoms.

The molds and samples were then placed in a covered container and low pressure steam introduced for 30 minutes maintaining a temperature of about 100° C. The samples were then removed from the molds, washed in cold water, bleached, washed and dried.

To determine tenacity, a strip of the product 2.54 cm. x 4.81 cm. long x about 0.6 cm. thick was cut, saturated with water, excess water removed, and broken on an Instron tester. Cross-head speed was about 1.27 cm./min., gage length 1.27 cm. and chart speed 12.7 cm./min. with a full scale reading of 25,000 g. The denier of the strip was calculated, in accordance with textile practice, as the weight in grams of 9,000 meters and tenacity was reported as grams to break/denier  $\times 10$ . The results obtained are shown in Table 1.

To illustrate the relation between maximum swelling concentration of NaOH and concentration at which maximum tenacity is attained, the figures set out in Table 1 were plotted and smooth curves drawn through them. These curves appear in FIG. 1 and as will be seen from

that figure, the concentration at which maximum swelling occurs coincides almost exactly with that at which maximum tenacity is obtained.

Table 1

| Percent free NaOH | Percent Contraction | Tenacity (g./d. $\times 10$ ) |
|-------------------|---------------------|-------------------------------|
| 4.75              | -----               | 0.74                          |
| 5.65              | -3                  | -----                         |
| 5.80              | -2.5                | 0.62                          |
| 6.49              | -----               | 0.91                          |
| 6.88              | -3.1                | -----                         |
| 7.09              | -----               | 1.01                          |
| 7.0               | -----               | 1.14                          |
| 7.8               | -----               | 1.46                          |
| 7.9               | -----               | 1.46                          |
| 7.95              | -2.8                | -----                         |
| 8.32              | -3.0                | -----                         |
| 8.30              | -----               | 0.97                          |
| 9.08              | -2.5                | -----                         |
| 9.4               | -----               | 1.10                          |
| 9.5               | -----               | 1.10                          |
| 9.6               | -----               | 1.16                          |
| 9.8               | 1.5                 | -----                         |
| 10.0              | -----               | 1.04                          |
| 10.3              | -0.6                | -----                         |
| 10.9              | 4.4                 | -----                         |
| 11.0              | -----               | 2.07                          |
| 11.7              | -0.6                | 0.89                          |
| 12.4              | 0.7                 | 0.69                          |

#### EXAMPLE II

The procedure of Example I was repeated using ramie fiber. The results obtained are given in Table 2 below and are plotted in FIG. 2. Again maximum swelling concentration corresponds remarkably well to maximum tenacity.

Table 2

| Free NaOH, Percent | Percent Contraction | Tenacity |
|--------------------|---------------------|----------|
| 6                  | 0                   | -----    |
| 7                  | 0                   | -----    |
| 8                  | 1                   | 0.56     |
| 8.6                | -----               | 0.53     |
| 9                  | 4.4                 | 0.72     |
| 9.5                | -----               | 0.60     |
| 10                 | 11.5                | 0.86     |
| 10.5               | -----               | 1.10     |
| 11.0               | 16.0                | 0.58     |
| 11.4               | -----               | 0.56     |
| 12.0               | 15.5                | 0.62     |
| 12.4               | -----               | 0.48     |
| 13                 | 14.8                | -----    |
| 14                 | 12.4                | -----    |

#### We claim:

In the manufacture of cellulose sponge wherein viscose, cellulose reinforcing fibers selected from the group consisting of cotton and ramie, and a pore-forming substance are combined to form a sponge mix, which is thereafter coagulated and regenerated to form a sponge structure, the improvement which comprises adding sodium hydroxide to said mix in an amount to bring the free sodium hydroxide concentration in said mix to between about 9 and about 12% by weight and to within about 1% of that necessary to cause maximum swelling of the fiber, said additive also being present in a proportion such as to increase the tenacity of the sponge structure to at least 30% more than that of a sponge made from said mix without said addition of sodium hydroxide.

#### References Cited in the file of this patent

#### UNITED STATES PATENTS

- |           |         |                |
|-----------|---------|----------------|
| 1,974,393 | Mostny  | Sept. 18, 1934 |
| 2,112,576 | Richter | Mar. 29, 1938  |
| 2,853,395 | Osborn  | Sept. 23, 1958 |